

March 24, 1970

D. S. DABKOWSKI ET AL

3,502,462

NICKEL, COBALT, CHROMIUM STEEL

Filed Nov. 29, 1965



INVENTORS.  
DONALD S. DABKOWSKI,  
PAUL J. KONKOL,  
LEW F. PORTER and  
ALLAN M. RATHBONE  
By *Donald S. Dalton*  
Attorney

1

3,502,462

**NICKEL, COBALT, CHROMIUM STEEL**

Donald S. Dabkowski, Pittsburgh, Paul J. Konkol, Plum Borough, Lew F. Porter, Monroeville Borough, and Allan M. Rathbone, Franklin Township, Westmoreland County, Pa., assignors to United States Steel Corporation, a corporation of Delaware

Filed Nov. 29, 1965, Ser. No. 510,341

Int. Cl. C22c 39/20, 39/50, 39/10

U.S. Cl. 75—128

1 Claim

**ABSTRACT OF THE DISCLOSURE**

A steel of high yield strength and good notch toughness adapted for use in wrought form as well as weld filler metal has the essential composition, by weight: nickel 9.5–14%; cobalt 6–10%; carbon 0.06–0.16%; molybdenum 0.7–1.5%; chromium .5–3%; and the balance iron except for residuals and minor impurities.

This invention relates to high yield strength steels having good notch toughness and to high yield strength weld metal of comparable properties.

In many applications where weight of the structure or thickness of the material must be maintained at a minimum, steels combining high yield strength and good notch toughness are required. Among the uses for which such steels are particularly suitable are the construction of pressure vessels, missile motor cases, submarine hulls, nuclear reactor pressure vessels and highly stressed structural members. Inasmuch as such uses require welding operations, it is also essential that the whole weldment including the weld metal possess superior properties.

There is an urgent need for high-toughness filler metals for joining constructional alloy steels with yield strengths in the range 160 to 220 K s.i. Such filler metals, after deposition by conventional fusion welding processes, must have high toughness and yield strengths approximately equal to those of the base steel in either the as-welded condition or after a relatively simple postweld heat treatment.

Two types of filler metals have been used to join high-yield-strength constructional alloys in the yield-strength range 160 to 220 K s.i. One group of filler metals, the maraging alloy steels, can be used to produce deposited and aged weld metal with satisfactory yield strengths but with only marginal toughness (30 to 50 ft.-lbs. Charpy V-notch energy absorption at 0° F.). Moreover, the maraging filler metals are not particularly compatible with conventional carbon-containing alloy steels. The second group of filler metals, carbon-containing nickel alloy steels, are generally used in the as-welded condition and exhibit moderately good toughness (40 to 60 ft.-lbs. Charpy V-notch energy absorption at 0° F.). However, to achieve a yield strength of 160 K s.i. and higher, these nickel alloy steels must contain about 0.20 to 0.30 percent carbon and, as a result, such alloys exhibit a moderately high susceptibility to weld cracking.

In the past several years, considerable data have been obtained on the yield strength-notch toughness relationship of a variety of alloy steels. These data indicate that there is an upper limit to the notch toughness of such steels. Moreover, it has been found that the notch-toughness limit decreases as the yield strength increases, particularly in steels with strength levels of 160 K s.i. or greater. In these high strength steels, the upper limit of notch toughness is about 60 ft.-lbs. (Charpy V-notch energy absorption at 0° F.) at 180 K s.i., and drops below 40 ft.-lbs. (Charpy V-notch energy absorption at 0° F.) at 200 K s.i.

2

Studies compiled by the Naval Research Laboratory have established an upper boundary strength-to-toughness curve for conventional high yield strength steels. The results of the study have been published in NRL Report 6300, June 1965, available from the Clearinghouse for Federal Scientific and Technical Information (CFSTI), Sills Building, 5285 Port Royal Road, Springfield, Va.

The present invention involves high strength steel having notch toughness in excess of the above mentioned limits and generally having a yield strength-to-toughness relationship which is better than conventional high yield strength steels. Steels according to the invention combine the strengthening principles of quenched and tempered steels with the strengthening principles of maraging steels and thus obtain a part of the strengthening from carbide precipitation and a part from precipitation of intermetallic compounds. Such steels exhibit the advantages of both quenched and tempered and maraging steels without the accompany disadvantages of these types of steels. Moreover, weld metal of such compositions combine the resistance to weld cracking of low carbon maraging steels with the superior toughness of nickel-cobalt steels.

Quenched and tempered steels require a carbon content in excess of about 0.2% to exhibit yield strength in 160 to 200 K s.i. range. At this carbon level, weldability is poor because the steel is subject to excessive cracking in the zone affected by weld heat and the maximum notch toughness obtainable is limited because of the brittleness of the carbides that strengthen these steels. However, the production of carbon-containing quenched and tempered steels is economical and such steels are commonly used for a variety of applications.

Maraging steels are essentially carbon free and obtain strength from the precipitation of complex nickel-molybdenum and nickel-titanium intermetallic compounds and obtain additional strength from undetermined mechanisms involving molybdenum and cobalt. Higher levels of yield strength and notch toughness can be developed in maraging steels because of the superiority of the strengthening mechanisms in these steels over the carbide precipitation strengthening mechanism in the quenched and tempered steels. However, because of the presence of titanium and aluminum in the maraging steels, care must be taken during melting to obtain the lowest possible levels of carbon, sulphur, nitrogen and oxygen. This is necessary to prevent the formation of particularly harmful particles of  $TiC$ ,  $TiS$ ,  $TiN$ ,  $AlN$ ,  $TiO_2$ ,  $Al_2O_3$  which adversely affect notch toughness. Thus, melting practices for maraging steels are relatively expensive and time consuming and special vacuum melting practices are required to develop optimum properties.

The present invention concerns a steel composition and weld metal for joining members thereof in which a part of the strengthening is obtained by the formation of nickel-molybdenum intermetallic compounds and part by the strengthening effects of cobalt. In these steels, it is possible to reduce the carbon content to below about 0.16% and thereby obtain good notch toughness. At this carbon level, some strengthening will result from the formation of carbides but the carbon content will not be so high that the weldability and notch toughness will be adversely affected. Such steels attain yield strength levels greater than 160 K s.i. but will not be as sensitive to the level of residual elements sulfur, nitrogen and oxygen, as are the maraging steels because these steels are substantially free of titanium and aluminum which are primarily responsible for the aforementioned harmful sulfides, carbides and nitrides. Weld metal of our steel compositions, quite unexpectedly, has a yield strength and toughness at least as good as the wrought forms.

According to the invention, there is provided a steel with high yield strength and good notch toughness which consists essentially of at least 9.5% nickel, preferably 9.5 to 14% nickel, at least 6% cobalt, preferably 6 to 10% cobalt, about 0.06 to 0.16% carbon, preferably 0.1 to 0.16% carbon, about 0.7 to 1.5% molybdenum, 0.5 to 3% chromium, preferably 1 to 2% chromium, and the balance substantially iron. The expression "substantially iron" means that the steels may contain small amounts, e.g. less than about 0.7% total of other elements such as 10

it is particularly important to control the nickel and cobalt contents of the steel if toughness-to-yield strength relationships exceeding conventional high yield strength steels are to be obtained.

5 The invention will be more fully understood by the following discussion and examples.

A number of samples of different composition were prepared and the check analysis, in percent by weight (used throughout herein), of these compositions is given in Table I.

TABLE I

| Steel: | C    | Mn    | P      | S     | Si    | Ni    | Cr    | Mo    | Co   | Al <sup>1</sup> | N     | O      |
|--------|------|-------|--------|-------|-------|-------|-------|-------|------|-----------------|-------|--------|
| A..... | 0.14 | 0.001 | 0.001  | 0.007 | 0.10  | 10.10 | 0.98  | <0.01 | 7.82 | 0.003           | 0.002 | 0.0029 |
| B..... | 0.15 | 0.006 | 0.001  | 0.007 | 0.093 | 10.10 | <0.10 | 1.00  | 8.03 | 0.003           | 0.002 | 0.0012 |
| C..... | 0.19 | 0.001 | <0.001 | 0.006 | 0.092 | 10.00 | <0.10 | <0.01 | 7.36 | 0.010           | 0.002 | 0.0004 |
| D..... | 0.11 | 0.010 | 0.0016 | 0.006 | 0.090 | 10.10 | 0.02  | 0.99  | 7.57 | 0.002           | 0.002 | 0.0017 |
| E..... | 0.12 | 0.004 | 0.0013 | 0.006 | 0.11  | 10.20 | 1.98  | 1.00  | 8.07 | 0.002           | 0.001 | 0.0027 |
| F..... | 0.12 | 0.007 | 0.0016 | 0.008 | 0.11  | 10.10 | 1.14  | 1.93  | 8.10 | 0.003           | 0.001 | 0.0031 |
| G..... | 0.16 | 0.004 | 0.0016 | 0.006 | 0.095 | 10.10 | 1.96  | 1.00  | 8.02 | 0.003           | 0.001 | 0.0017 |
| H..... | 0.20 | 0.010 | 0.003  | 0.008 | 0.087 | 10.10 | 1.91  | 1.00  | 7.94 | 0.003           | 0.002 | -----  |
| I..... | 0.11 | 0.004 | 0.001  | 0.007 | 0.088 | 10.00 | 1.02  | 1.00  | 6.03 | 0.006           | 0.002 | 0.0010 |
| J..... | 0.11 | 0.004 | 0.0011 | 0.007 | 0.096 | 9.84  | 1.95  | 0.91  | 5.94 | 0.002           | .001  | 0.0024 |

<sup>1</sup> Acid soluble.

manganese, silicon and aluminum, (the latter up to about 0.025% max.) to perform their common functions and residual amounts of sulfur and phosphorous. The preferred composition is a steel which consists essentially of 9.5 to 12% nickel, 6 to 10% cobalt, 0.1 to 0.16% carbon, 0.7 to 1.5% molybdenum, 1 to 2% chromium and the balance substantially iron. It has been found that

30

Samples of these compositions were strengthened by austenitizing, water quenching and aging in a conventional manner and then subjected to mechanical property evaluation. The results of this evaluation and a comparison of these results with the properties of as-quenched samples are presented in Table II.

TABLE II

| Steel: | Aging temp., °F. <sup>1</sup> | Yield strength (0.2% offset), K.s.i. | Tensile strength, K.s.i. | Elongation in 1 inch, percent | Reduction of area, percent | Hardness, $R_C$ |       | Charpy V-notch energy absorption, ft.-lb. |  |
|--------|-------------------------------|--------------------------------------|--------------------------|-------------------------------|----------------------------|-----------------|-------|-------------------------------------------|--|
|        |                               |                                      |                          |                               |                            | +80° F.         | 0° F. |                                           |  |
| A..... | As-quenched                   | 166                                  | 211                      | 17.0                          | 66.3                       | 45.5            | 56    | 48                                        |  |
|        | 400                           | 164                                  | 207                      | 16.0                          | 65.9                       | 46.0            | 50    | 53                                        |  |
|        | 600                           | 167                                  | 192                      | 16.0                          | 68.3                       | 44.0            | 52    | 50                                        |  |
|        | 800                           | 168                                  | 181                      | 16.0                          | 66.8                       | 42.0            | 54    | 42                                        |  |
|        | 900                           | 156                                  | 162                      | 19.0                          | 70.2                       | 39.0            | 84    | 65                                        |  |
|        | 1,000                         | 131                                  | 140                      | 22.0                          | 74.9                       | 34.0            | 124   | 124                                       |  |
|        | 1,100                         | 112                                  | 130                      | 24.0                          | 76.7                       | 30.0            | 157   | 141                                       |  |
|        | 1,200                         | 99                                   | 138                      | 24.0                          | 73.0                       | 31.5            | 131   | 130                                       |  |
| B..... | As-quenched                   | 170                                  | 228                      | 6.0                           | 10.4                       | 48.5            | 4     | 4                                         |  |
|        | 400                           | 180                                  | 226                      | 5.0                           | 9.0                        | 48.5            | 4     | 4                                         |  |
|        | 600                           | 186                                  | 211                      | 5.5                           | 13.8                       | 46.5            | 4     | 4                                         |  |
|        | 800                           | 187                                  | 206                      | 5.0                           | 16.2                       | 45.5            | 4     | 4                                         |  |
|        | 900                           | 191                                  | 205                      | 5.0                           | 9.7                        | 50.0            |       |                                           |  |
|        | 1,000                         | 202                                  | 209                      | 4.0                           | 10.5                       | 47.0            | 4     | 3                                         |  |
|        | 1,100                         | 154                                  | 156                      | 2.0                           | 5.6                        | 39.0            | 3     | 2                                         |  |
|        | 1,200                         | 114                                  | 162                      | 9.5                           | 11.6                       | 37.0            | 5     |                                           |  |
| C..... | As-quenched                   | 172                                  | 233                      | 8.0                           | 22.8                       | 49.5            | 6     | 5                                         |  |
|        | 400                           | 189                                  | 223                      | 11.0                          | 39.0                       | 48.0            | 5     | 5                                         |  |
|        | 600                           | 178                                  | 189                      | 12.0                          | 50.5                       | 44.5            | 7     | 3                                         |  |
|        | 800                           | 145                                  | 149                      | 16.0                          | 55.7                       | 36.0            | 12    | 9                                         |  |
|        | 900                           | 128                                  | 133                      | 19.5                          | 60.1                       | 31.0            | 20    | 15                                        |  |
|        | 1,000                         | 117                                  | 121                      | 23.0                          | 65.1                       | 27.0            | 34    | 26                                        |  |
|        | 1,100                         | 103                                  | 113                      | 28.5                          | 66.4                       | 25.0            | 53    | 45                                        |  |
|        | 1,200                         | 87                                   | 145                      | 19.0                          | 18.5                       | 31.5            | 13    | 11                                        |  |
| D..... | As-quenched                   | 158                                  | 207                      | 17.0                          | 65.3                       | 44.5            | 50    | 47                                        |  |
|        | 400                           | 164                                  | 201                      | 17.0                          | 66.4                       | 45.0            | 51    | 51                                        |  |
|        | 600                           | 171                                  | 199                      | 16.0                          | 62.2                       | 44.5            | 46    | 44                                        |  |
|        | 800                           | 172                                  | 199                      | 18.0                          | 65.2                       | 44.5            | 42    | 39                                        |  |
|        | 900                           | 183                                  | 203                      | 17.0                          | 67.7                       | 46.0            | 50    | 49                                        |  |
|        | 1,000                         | 180                                  | 191                      | 16.5                          | 70.8                       | 44.5            | 56    | 60                                        |  |
|        | 1,100                         | 137                                  | 151                      | 22.0                          | 75.4                       | 35.0            | 121   | 111                                       |  |
|        | 1,200                         | 114                                  | 155                      | 21.0                          | 72.8                       | 35.0            | 112   | 110                                       |  |
| E..... | As-quenched                   | 158                                  | 208                      | 16.0                          | 65.9                       | 45.5            | 56    | 58                                        |  |
|        | 400                           | 155                                  | 198                      | 16.0                          | 67.9                       | 45.0            | 64    | 69                                        |  |
|        | 600                           | 159                                  | 193                      | 16.0                          | 67.8                       | 49.0            | 60    | 61                                        |  |
|        | 800                           | 171                                  | 204                      | 17.0                          | 66.5                       | 46.0            | 51    | 46                                        |  |
|        | 900                           | 184                                  | 207                      | 16.0                          | 67.7                       | 47.0            | 58    | 60                                        |  |
|        | 1,000                         | 172                                  | 181                      | 18.0                          | 71.7                       | 41.5            | 87    | 88                                        |  |
|        | 1,100                         | 14                                   | 149                      | 22.0                          | 75.2                       | 35.5            | 122   | 125                                       |  |
|        | 1,200                         | 105                                  | 148                      | 21.0                          | 74.4                       | 33.5            | 130   | 129                                       |  |
| F..... | As-quenched                   | 177                                  | 228                      | 14.0                          | 55.2                       | 48.0            | 22    | 22                                        |  |
|        | 400                           | 104                                  | 227                      | 15.0                          | 58.6                       | 47.0            | 24    | 24                                        |  |
|        | 600                           | 195                                  | 222                      | 14.5                          | 56.8                       | 47.5            | 21    | 20                                        |  |
|        | 800                           | 206                                  | 229                      | 14.0                          | 56.4                       | 48.0            | 21    | 20                                        |  |
|        | 900                           | 207                                  | 223                      | 16.0                          | 59.6                       | 48.5            | 21    | 19                                        |  |
|        | 1,000                         | 186                                  | 190                      | 16.0                          | 61.0                       | 43.0            | 27    | 24                                        |  |
|        | 1,100                         | 132                                  | 152                      | 21.0                          | 69.1                       | 35.0            | 54    | 48                                        |  |
|        | 1,200                         | 114                                  | 149                      | 20.0                          | 68.8                       | 34.0            | 71    | 66                                        |  |

TABLE II—Continued

| Aging<br>temp., °F. <sup>1</sup> | Yield<br>strength<br>(0.2%<br>offset),<br>K s.i. | Tensile<br>strength,<br>K s.i. | Elongation<br>in 1 inch,<br>percent | Reduction<br>of area,<br>percent | Hard-<br>ness,<br>R <sub>c</sub> | Charpy V-notch<br>energy absorption,<br>ft.-lb. |       |     |
|----------------------------------|--------------------------------------------------|--------------------------------|-------------------------------------|----------------------------------|----------------------------------|-------------------------------------------------|-------|-----|
|                                  |                                                  |                                |                                     |                                  |                                  | +80° F.                                         | 0° F. |     |
| G -----                          | As-quenched                                      | 184                            | 236                                 | 15.0                             | 64.3                             | 50.0                                            | 38    | 41  |
|                                  | 400                                              | 176                            | 224                                 | 16.0                             | 65.6                             | 47.0                                            | 43    | 40  |
|                                  | 600                                              | 177                            | 214                                 | 16.0                             | 65.0                             | 47.0                                            | 35    | 35  |
|                                  | 800                                              | 184                            | 223                                 | 17.0                             | 65.3                             | 48.0                                            | 32    | 33  |
|                                  | 900                                              | 203                            | 227                                 | 16.0                             | 66.9                             | 49.0                                            | 40    | 37  |
|                                  | 1,000                                            | 185                            | 191                                 | 17.5                             | 71.1                             | 45.0                                            | 63    | 62  |
|                                  | 1,100                                            | 142                            | 161                                 | 22.0                             | 74.6                             | 38.0                                            | 104   | 105 |
|                                  | 1,200                                            | 120                            | 158                                 | 21.0                             | 73.0                             | 36.0                                            | 109   | 104 |
| H -----                          | As-quenched                                      | 199                            | 263                                 | 14.5                             | 56.4                             | 51.0                                            | 20    | 18  |
|                                  | 400                                              | 190                            | 242                                 | 14.0                             | 58.7                             | 50.0                                            | 24    | 24  |
|                                  | 600                                              | 199                            | 243                                 | 15.0                             | 57.3                             | 50.5                                            | 20    | 16  |
|                                  | 800                                              | 215                            | 251                                 | 16.0                             | 59.1                             | 51.5                                            | 22    | 20  |
|                                  | 900                                              | 185                            | 202                                 | 16.0                             | 67.4                             | 44.0                                            | 43    | 38  |
|                                  | 1,000                                            | 137                            | 169                                 | 20.5                             | 69.6                             | 39.5                                            | 72    | 66  |
|                                  | 1,200                                            | 119                            | 165                                 | 21.0                             | 70.3                             | 37.0                                            | 72    | 69  |
| I -----                          | As-quenched                                      | 165                            | 212                                 | 16.0                             | 65.6                             | 46.5                                            | 50    | 49  |
|                                  | 400                                              | 172                            | 206                                 | 15.0                             | 67.4                             | 46.0                                            | 54    | 52  |
|                                  | 600                                              | 173                            | 201                                 | 16.0                             | 66.5                             | 45.0                                            | 47    | 43  |
|                                  | 800                                              | 177                            | 200                                 | 16.0                             | 65.7                             | 46.0                                            | 46    | 44  |
|                                  | 900                                              | 181                            | 199                                 | 16.0                             | 68.2                             | 46.0                                            | 58    | 53  |
|                                  | 1,000                                            | 177                            | 189                                 | 18.0                             | 72.3                             | 44.5                                            | 68    | 70  |
|                                  | 1,100                                            | 135                            | 149                                 | 22.0                             | 77.1                             | 36.0                                            | 121   | 114 |
|                                  | 1,200                                            | 112                            | 155                                 | 22.0                             | 71.6                             | 36.0                                            | 109   | 106 |
| J -----                          | As-quenched                                      | 153                            | 200                                 | 16.0                             | 67.2                             | 44.0                                            | 65    | 68  |
|                                  | 400                                              | 151                            | 190                                 | 17.0                             | 67.9                             | 43.0                                            | 74    | 75  |
|                                  | 600                                              | 153                            | 186                                 | 17.0                             | 67.5                             | 42.0                                            | 69    | 68  |
|                                  | 800                                              | 161                            | 191                                 | 18.0                             | 68.2                             | 44.0                                            | 65    | 61  |
|                                  | 900                                              | 171                            | 194                                 | 18.0                             | 68.7                             | 44.0                                            | 74    | 73  |
|                                  | 1,000                                            | 163                            | 173                                 | 20.0                             | 72.2                             | 40.0                                            | 96    | 98  |
|                                  | 1,100                                            | 126                            | 145                                 | 22.0                             | 77.0                             | 33.0                                            | 142   | 143 |
|                                  | 1,200                                            | 108                            | 145                                 | 21.0                             | 74.6                             | 34.0                                            | 139   | 147 |

<sup>1</sup>1/2-inch-thick plate samples austenitized at 1,500° F. for 1 hour and water-quenched, then aged for 5 hours at the indicated temperature, and water-quenched.

The results reported in Table II show that both chromium and molybdenum are necessary in the high nickel-cobalt steels to obtain good notch toughness (samples A, B, C and D) and that changes in chromium content within the 1 to 2% range have little effect on the yield strength and notch toughness of these steels except that at equivalent strengths, the 2% chromium-1% molybdenum steel exhibited about a 10 ft.-lb. higher Charpy V-notch energy absorption at 0° F. (samples D and E).

It is also noted that the yield strength at the peak aging temperature of 900° F. increased from 184 to 203 K s.i. when the carbon was increased from 0.12 to 0.2% and the notch toughness decreased progressively from about 60 ft.-lbs. (Charpy V-notch) for the 0.12% carbon sample to about 20 ft.-lbs. in the 0.2% carbon samples (samples E, G and H). Changes in the cobalt content from 6 to 8% have little effect on the strength and toughness of the high nickel-chromium-molybdenum steel (samples D and I), but steels with 8% cobalt are superior to steels with 6% cobalt and 2% chromium (samples E and J).

One unusual feature of our steels is the manner in which the notch toughness starts to increase at aging temperatures below those at which the yield strength reaches its peak. This is contrary to the behavior of conventional quenched and tempered steels and is indirect evidence that the strengthening mechanism described in our steels is different from that involved in conventional quenched and tempered steels. The increasing toughness at aging temperatures of 900 to 1000° F. makes it possible to obtain still better combinations of strength and toughness.

It is also apparent from the data in Table II that a strong aging peak occurs at an aging temperature of 900° F. This is the optimum aging temperature for maraging steels and thus provides indirect evidence that the strengthening mechanisms operating in our steels are similar to those operating in maraging steels as well. It is also observed that at the peak aging temperature, the increase in strength realized from an increase in carbon content of from 0.16 to 0.20% is less than the increase in strength realized from an increase in carbon of from 0.12 to 0.16%. This indicates that the optimum carbon content is no higher than 0.16% C.

It is also apparent from Table II that steels according

to the invention are capable of achieving a notch toughness of about 100 ft.-lbs. (Charpy V-notch energy at 0° F.) at a yield strength of 160 K s.i. and over 60 ft.-lbs. at a yield strength of over 180 K s.i. These levels of notch toughness are substantially higher than those obtained in quenched and tempered steels strengthened primarily by carbide precipitation.

Of considerable importance, however, is the discovery that it is necessary to maintain controlled nickel and cobalt contents to provide a steel with yield strength-to-toughness relationships better than conventional high strength steels. As discussed above, studies of previous investigators compiled by the Naval Research Laboratory have established an upper boundary curve for conventional high yield strength steels. This curve is reproduced in FIGURE 1 and shows the aforementioned upper boundary limit of the strength and toughness of conventional steels in the range of 170 to 200 K s.i. Also shown in FIGURE 1 are the yield strength and notch toughness of each of five steel compositions which differed only in nickel and cobalt contents. Compositions of these samples are shown in Table III.

55

TABLE III

| Steel  | Ni   | Co   | C   | Mn    | P    | S     | Si   | Cr   | Mo   | A    |
|--------|------|------|-----|-------|------|-------|------|------|------|------|
| L----- | 12.0 | 8.0  | .12 | >0.02 | 0.01 | 0.005 | 0.10 | 2.00 | 1.00 | .003 |
| M----- | 10.0 | 8.0  | .12 | 0.02  | 0.01 | 0.005 | 0.10 | 2.00 | 1.00 | .003 |
| N----- | 9.0  | 8.0  | .12 | 0.02  | 0.01 | 0.005 | 0.10 | 2.00 | 1.00 | .003 |
| P----- | 10.0 | 10.0 | .12 | 0.02  | 0.01 | 0.005 | 0.10 | 2.00 | 1.00 | .003 |
| R----- | 10.0 | 5.0  | .12 | 0.02  | 0.01 | 0.005 | 0.10 | 2.00 | 1.00 | .003 |

As can be seen from FIGURE 1, steels containing 9% nickel with 8% cobalt (sample N) and steels containing 10% nickel but only 5% cobalt (sample R) possessed a strength-to-toughness relationship below the upper boundary curve for conventional high yield strength steels. In contrast, the steels in which the nickel was maintained above 9.5% and the cobalt at 6% or greater have yield strength and toughness exceeding the upper boundary curve (samples L, M and P).

At least 9.5% nickel is believed to be necessary to provide sufficient nickel so that strengthening through precipitation of nickel-molybdenum compound (Ni<sub>3</sub>Mo) will occur. It has also been found that chromium contents

65

60

70

amounts of from 1 to 2% are desirable in these alloys to obtain high notch toughness at high yield strengths and that molybdenum contents of 2.0% are in excess of the optimum level for good notch toughness in steels of this type.

As is known, the properties of metals can be generally improved by metallurgical practices which include hot and cold working and various heat treatments. Thus, wrought forms of steel typically have the best properties. It is, therefore, quite surprising to discover that as a weld-filler metal the steel compositions within the purview of the invention possess mechanical properties as good as or better than wrought samples. Welding involves coalescing metal that is melted by local application of heat whereby a base metal and filler metal are fused together. We have found that weld metal of the steel compositions according to the invention, containing at least 9.5% nickel, preferably 9.5 to 12% nickel, at least 6% cobalt, preferably 6 to 10% cobalt, 0.5 to 3% chromium, 0.7 to 1.5% molybdenum, 0.06 to 0.16% carbon and the balance substantially iron, can be made which possesses yield strengths greater than 160 K.s.i. and notch toughness of 70 ft.-lbs. or greater (Charpy V-notch energy absorption at 0° F.). The weld metal may also contain small amounts, i.e. up to about 0.7% total, of other elements such as manganese, silicon and aluminum (the latter up to about 0.025%) to perform their common functions, and residual amounts of phosphorous and sulfur. When used as a weld-filler metal, a preferred composition consists essentially of 9.5 to about 10% nickel, 6 to about 8% cobalt, 0.1 to 0.16% carbon, about 1 to 2% chromium, .7 to 1.25% molybdenum and the balance substantially iron.

The following examples typical of the improved weld-filler metal according to the invention. Samples of weld metal of each of four compositions shown in Table IV were prepared.

TABLE IV

| Item | C    | Mn    | P     | S     | Si   | Ni   | Co   | Cr   | Mo   | Al    |
|------|------|-------|-------|-------|------|------|------|------|------|-------|
| W    | 0.10 | 0.010 | 0.002 | 0.006 | 0.09 | 10.1 | 8.25 | 1.02 | 1.01 | 0.002 |
| X    | 0.15 | 0.005 | 0.001 | 0.007 | 0.11 | 10.0 | 6.10 | 2.02 | 1.03 | 0.002 |
| Y    | 0.11 | 0.004 | 0.001 | 0.006 | 0.11 | 10.2 | 7.81 | 2.02 | 1.01 | 0.002 |
| Z    | 0.13 | 0.004 | 0.001 | 0.006 | 0.09 | 10.0 | 6.11 | 1.02 | 1.04 | 0.001 |

Weld metal or compositions W and Y were tested in both the unaged and aged condition and weld metal of compositions X and Z were tested after aging at 900° F. for 5 hours. The mechanical properties are reported in Table V and, for comparison, the mechanical properties of plate samples of these same compositions are also included.

bare wires and inert-gas-shielded tungsten-arc welding.

Weld filler metal of our composition may be used in the as-deposited condition if a yield strength on the low side of the 160 to 220 K.s.i. range is desired. When maximum strength is required, a simple post weld aging treatment may be used. Aging is not critical and normal aging practices for the base metal can be used.

When weldments are to be made on plates or sheets of similar compositions, a filler wire of the same composition can also be used. If, however, a different steel base is to be welded then the composition of the filler wire should be selected so that, after mixing with the base and taking reactions with the atmosphere into account, a weld metal with the required composition is produced.

It is desirable to maintain the carbon content of the weld metal at between about 0.10 to 0.16% to develop the best strength levels with minimum loss in crack resistance and toughness. Manganese, silicon, and aluminum should be maintained at the lowest levels consistent with the good deoxidation of the molten weld pool because increases in these elements cause a loss in toughness. Both phosphorous and sulfur should be maintained at low levels because both elements reduce toughness and increase susceptibility to hot shortness. The nickel content should be at least 9.5%, preferably about 10% because a decrease causes a loss in hardenability and also a less potent hardening reaction to occur upon postweld aging. An increase in nickel over about 10% increases the tendency to form retained austenite which, in turn, decreases both strength and toughness; however, up to about 12% nickel is satisfactory. The cobalt content should be at least 6%, preferably about 6 to 8% because cobalt causes a strength increase and also increases the temperature of martensite formation which, in turn, increases the resistance to weld cracking. Large amounts of cobalt, however, e.g. over about 10%, cause an undesirable loss in toughness and hardenability.

Although the effects are not well understood, chromium contents in the range 1.0 to 2.0% appear to be beneficial in that the strength is increased with no apparent loss in toughness. The optimum molybdenum content is about 0.7 to 1.25%, preferably 1.0%; at levels lower than 1.0%, an insufficient age-hardening reaction may occur, and at levels significantly higher than 1.5%, a severe loss in toughness will occur.

In view of the foregoing, it is apparent that various changes and modifications may be made within the purview of the invention and, accordingly, the scope of the

TABLE V

| Steel: | Postweld heat treatment                                      | Yield strength (0.2% offset), K.s.i. | Tensile strength, K.s.i. | Elongation in 1 inch, percent | Charpy V-notch energy reduction absorption, ft.-lb. |       |
|--------|--------------------------------------------------------------|--------------------------------------|--------------------------|-------------------------------|-----------------------------------------------------|-------|
|        |                                                              |                                      |                          |                               | +80° F.                                             | 0° F. |
| W      | None (unaged)                                                | 170                                  | 198                      | 16.0                          | 50                                                  | 61    |
| W      | Rolled plate, austenitized and quenched                      | 158                                  | 207                      | 17.0                          | 65.3                                                | 50    |
| W      | 900° F./5 hrs                                                | 174                                  | 200                      | 18.0                          | 68                                                  | 53    |
| W      | Rolled plate, austenitized, quenched, and aged 900° F./5 hrs | 183                                  | 203                      | 17.0                          | 67.7                                                | 50    |
| X      | 900° F./5 hrs                                                | 187                                  | 223                      | 18.0                          | 66                                                  | 65    |
| X      | Rolled plate, austenitized, quenched, and aged 900° F./5 hrs | 192                                  | 217                      | 17.0                          | 66.6                                                | 41    |
| Y      | None (unaged)                                                | 172                                  | 206                      | 18.0                          | 67                                                  | 87    |
| Y      | Rolled plate, austenitized and quenched                      | 158                                  | 208                      | 16.0                          | 65.9                                                | 56    |
| Y      | 900° F./5 hrs                                                | 194                                  | 209                      | 18.5                          | 69                                                  | 93    |
| Y      | Rolled plate, austenitized, quenched, and aged 900° F./5 hrs | 184                                  | 207                      | 16.0                          | 67.7                                                | 58    |
| Z      | 900° F./5 hrs                                                | 189                                  | 214                      | 18.0                          | 67                                                  | 73    |
| Z      | Rolled plate, austenitized, quenched, and aged 900° F./5 hrs | 178                                  | 201                      | 18.0                          | 65.5                                                | 53    |

It is apparent from Table V above that the properties of the weld metal, unexpectedly, compare very favorably with those of rolled plate specimens. Conventional fusion welding can satisfactorily produce weldments and weld metal with superior properties. The data reported in Table V were obtained from weld metal deposited using solid

invention should be limited only by the appended claims.

We claim:

1. A steel having high yield strength and good notch toughness consisting essentially of 9.5% to 14% nickel, 6% to 10% cobalt, 0.06 to 0.16% carbon, 0.7 to 1.5% molybdenum, 0.5 to 3% chromium and the balance sub-

stantially iron except for residuals and incidental impurities.

**References Cited**

UNITED STATES PATENTS  
1,473,208 11/1923 Clement.

3,152,934 10/1964 Lula \_\_\_\_\_ 75—128,9  
3,285,738 11/1966 Johnson \_\_\_\_\_ 75—128  
3,366,471 1/1968 Hill.

5 HYLAND BIZOT, Primary Examiner

UNITED STATES PATENT OFFICE  
CERTIFICATE OF CORRECTION

Patent No. 3,502,462

March 24, 1970

Donald S. Dabkowski et al.

It is certified that error appears in the above identified patent and that said Letters Patent are hereby corrected as shown below:

Column 2, line 20, "accompany" should read -- accompanying --. Columns 3 and 4, TABLE II, Steel B, last line under heading "0° F", insert -- 5 --; Steel E, line 7, under heading "Yield Strength . . ." "1 4" should read -- 134 --; Steel G, line 1 of "Reduction of area, percent" should read -- 64.3 --. Column 6, line 43, "conventional" should read -- conventional --. Columns 5 and 6, TABLE III, last column in the heading, "A" should read -- A1 --. Column 7, line 27, "well" should read -- weld --.

Signed and sealed this 22nd day of December 1970.

(SEAL)

Attest:

Edward M. Fletcher, Jr.

Attesting Officer

WILLIAM E. SCHUYLER, JR.

Commissioner of Patents

**Notice of Adverse Decision in Interference**

In Interference No. 97,931 involving Patent No. 3,502,462, D. S. Dabkowski, P. J. Konkol, L. F. Porter and A. M. Rathbone, NICKEL, COBALT, CHROMIUM STEEL, final judgment adverse to the patentees was rendered Jan. 28, 1974, as to claim 1.

*[Official Gazette May 21, 1974.]*